

# UNITED STATES PATENT OFFICE.

EUGEN HURWITZ, OF BERLIN, GERMANY, ASSIGNOR, BY MESNE ASSIGNMENTS, TO  
GENERAL ELECTRIC COMPANY, A CORPORATION OF NEW YORK.

## MANUFACTURE OF METALLIC ILLUMINATING BODIES FOR ELECTRIC INCANDESCENT LAMPS.

1,099,704.

Specification of Letters Patent.

Patented June 9, 1914.

No Drawing.

Application filed October 16, 1906. Serial No. 339,165.

*To all whom it may concern:*

Be it known that I, EUGEN HURWITZ, a subject of the German Emperor, and a resident of Alte Jakobstrasse 139, Berlin, Germany, have invented certain new and useful Improvements in the Manufacture of Metallic Illuminating Bodies for Electric Incandescent Lamps; and I do hereby declare the following to be a full, clear, and exact 10 description of the invention, such as will enable others skilled in the art to which it app pertains to make and use the same.

My invention relates to an improved process for the manufacture of metallic illuminating bodies for electric incandescent lamps, said process resulting in a superior filament not heretofore produced.

In the manufacture of illuminating bodies from tungsten, by subjecting raw filaments 20 cemented together from finely divided particles to a sintering process very strong contraction takes place. This contraction immediately shortens the length of the final metallic filament as compared with the raw 25 filament and does not always take place uniformly, and the resistances of the illuminating bodies consequently fluctuate within certain limits. It has been found that this shriveling process proceeds more uniformly 30 if the filaments treated be subjected to a gentle pull or put under slight tension during the process by which they are caused to shrivel up. Means for effecting this pull or tension, loading of a stirrup or loop shaped 35 filament by a small weight attached to the stirrup or loop, are known of themselves and have been used for the purpose of drawing out filaments already finished into a pointed form.

40 The new process consists in acting upon or loading the raw filament while in the process of manufacture. By this means several advantages are secured. Firstly the disadvantage of irregular contraction already mentioned is avoided, the filament being characterized by a uniformity of contraction which results from the tension upon it while its particles are sintered and shrunk together. Moreover the straight portions 45 of the filament will be perfectly straight and the filament will present a similar evenness throughout. Filaments which have been fully sintered and finished without a load 50 cannot be entirely freed from irregularities

and kinks by subsequent tension treatment 55 as above referred to, no matter how highly they may be incandescent so that my new process gives to the filament characteristics of evenness by which it may readily be distinguished from filaments of a similar nature produced in any other known manner. In addition to this a considerable commercial advantage is attained inasmuch as a simplification of the manipulations required for the formation of the finished filament is 60 effected, as well as a saving in the plant required, in so far as the drawing of the filament into a pointed form does not necessitate a second operation in the case of filaments of this said pointed "hair pin" loop 65 form, the advantages of my invention are specially pronounced. Finally the number of defective and unserviceable filaments produced is materially lessened, as filaments which would be deformed during the sintering process in consequence of deficient quality or careless handling, without being loaded, yield when loaded serviceable finished filaments.

The process consists therefore broadly in 80 subjecting the raw filaments consisting of metallic particles while acted upon by a load to that process which turns them into finished filaments, so that the chemical and physical actions which convert the filament 85 to its final shape will take place while such filament is under the expanding or stretching action of the load. The load may consist of a small weight of any desired kind, conveniently of a small hook of metallic tungsten. This small weight or hook is hung within the loop of the raw filament and its gravity exerts a tension in a direction 90 away from the points of support for the raw filament. These raw filaments, being 95 composed as above described of finely divided particles of tungsten cemented together, are, of course, filaments incapable of use as incandescent filaments, being composed of fine tungsten particles and cementing material. Its physical make-up is composite and not uniform. If this raw filament is imagined to consist of a series of successive particles of tungsten, cement, etc., it becomes apparent that the small weight 100 would break the filament if the cement were removed at any one point. As the electric current passes through this raw filament, it

causes the removal of the cementing means without, however, breaking the continuity of the thread. The weight of the hook is, of course, so figured that it will not of its own weight and by mere force of weight break through the filament. The weight of the hook is relied upon to exercise a tension away from the points of support of the filament so that it assists in performing the unique function of producing a properly formed filament by a pull against the filament which results paradoxically in a metallic filament far shorter in length than the raw filament, and in spite of the pull or tension of the hook in a direction away from the points of support, it is nearer the points of support of the filament at the end of the process than at the beginning.

Having thus described my invention, what I claim as new therein and desire to secure by Letters Patent of the United States of America is:

1. The process for the manufacture of illuminating filaments of tungsten which consists in loading a very thin thread-like agglomeration of tungsten and carbon while in a very tender and brittle state in such a way that tension would be exerted upon said thread-like body in a direction away from its points of support and effecting the conversion of said raw agglomerated body into a finished metallic filament during the time that said load exercises effective tension upon the filamentary body.

2. The method for the manufacture of fil-

aments consisting of fine metallic particles sintered together which consists in subjecting raw filaments to treatment whereby the particles of the final filaments are sintered and shrunk together while the filaments are under tension.

3. The method which consists in subjecting raw filaments consisting of finely divided metallic particles sintered together to treatment whereby the cementing means is eliminated and the particles of the final material of the filament are sintered together while the filament is under tension.

4. An incandescent filamentary body consisting of particles of metallic tungsten uniformly sintered together by application of tension to the agglomerated metallic particles during the sintering operation into a coherent filament even throughout its length and perfectly straight except where definitely bent.

5. An incandescent body consisting of particles of metallic tungsten uniformly sintered and shrunk together by application of tension to the agglomerated metallic particles during the sintering operation into an even filament of loop shape having a sharp bend and straight even legs.

In testimony, that I claim the foregoing as my invention, I have signed my name in presence of two subscribing witnesses.

EUGEN HURWITZ.

Witnesses:

HENRY HASPER,  
WOLDEMAN HAUPT.